

March 2, 1954

D. C. BLAIR ET AL  
METHOD FOR INHIBITING ROLL PICKUP IN  
CONTINUOUS ANNEALING OF STEEL STRIP  
Filed Jan. 30, 1953

2,671,038

FIG. 1.



FIG. 2.



FIG. 3.



Inventors:  
DAVID C. BLAIR and  
HARRY F. SHANNON,  
Donald G. Dalton  
their Attorney.

Patented Mar. 2, 1954  
2,671,038

UNITED STATES PATENT OFFICE

**METHOD FOR INHIBITING ROLL PICKUP IN  
CONTINUOUS ANNEALING OF STEEL STRIP**

David C. Blair, Washington Township, Westmoreland County, and Harry F. Shannon, Mount Lebanon Township, Allegheny County, Pa., assignors to United States Steel Corporation, a corporation of New Jersey

Application January 30, 1953, Serial No. 334,224

1 Claim. (Cl. 148—16)

**1** This invention relates to the continuous heat-treatment of flat-rolled metal products and, in particular, to provisions for inhibiting the building up of accretions of oxides on the rolls which support the products during travel through a continuous annealing furnace.

Great difficulty has been experienced in the continuous annealing of ferrous strip, and particularly silicon-steel strip, because of the tendency of the furnace rolls over which the strip passes, to pick up adherent accretions of oxides which build up quickly to such a form and extent that they mark the strip in the manner known as "dimpling." The rolls are usually composed of ordinary steel or a heat-resistant alloy. Apparently, particles composed of the mixed oxides of iron and silicon adhere to the furnace conveyor rolls during the annealing process. As the annealing campaign progresses, these particles, commonly called "pick-up," increase in size to such an extent that the strip passing over the roll is marked or "dimpled" rendering it unsuitable for most applications. When this occurs, usually in from several hours to several days, depending on the composition of the furnace atmosphere, the furnace must be cooled to approximately room temperature and the particles removed from the rolls by mechanical means. A great loss of production results and the increased costs of processing thus involved are serious.

We have invented a novel method for inhibiting the pick-up of oxide particles by the furnace rolls, thus almost eliminating the necessity for periodically shutting down the furnace to clean the rolls or greatly reducing the frequency thereof. In a preferred practice, we discharge streams of reducing gas onto the surface of the strip ahead of the points of contact with the rolls. This not only prevents the formation of oxides but tends to reduce any oxides already formed on the strip and keeps the rolls free from accumulating accretions or pick-up. The preferred apparatus comprises a manifold or nozzle pipe disposed in the V between the body of the conveyor roll and strip approaching it. The pipe is connected to a supply of a suitable gas and is provided with nozzles or outlet ports spaced therealong, discharging into the V. Any reducing gas such as hydrogen, methane or carbon monoxide may be used for strip generally but, for silicon-steel strip, an atmosphere largely of hydrogen is preferable because the other gases mentioned tend to re-carburize the strip whereas decarburization is often an important objective of the annealing practice.

The general object of the invention is to provide a furnace for annealing flat metal products which will inhibit the formation of adherent accretions on the furnace rolls, and to provide a method for inhibiting the formation of adherent accretions on the furnace rolls.

Other objects and features of the invention will be apparent from the following detailed description and the accompanying drawings illustrating a preferred embodiment and a modification. In the drawings,

A complete understanding of the invention may be obtained from the following detailed description and explanation thereof which refer to the accompanying drawings illustrating a preferred embodiment and a modification. In the drawings,

Figure 1 is a central longitudinal section, largely diagrammatic, through a strip-annealing furnace embodying the apparatus adapted for carrying out the method of our invention;

Figure 2 is a partial vertical section taken along the plane of line II—II of Figure 1; and

Figure 3 is a transverse section through one of the conveyor rolls and its associated gas-supply pipe, taken along the plane of line III—III of Figure 2.

Referring in detail to the drawings and, for the present, to Figure 1, a strip-annealing furnace indicated generally at 10 comprises a refractory-lined enclosure laid up within a conventional binding fabricated from steel plate and rolled sections (not shown) in the known manner.

The furnace has an entrance opening 11 at one end and an exit opening 12 at the other,

adapted to permit the passage of strip therethrough from an uncoiler at the entrance end to a recoiler at the exit end.

The furnace may be heated by any suitable means, i. e., electric resistors, radiant combustion tubes or the like.

A controlled atmosphere, usually decarburizing, is supplied to the furnace chamber by any convenient means (not shown).

In order to maintain each point along the strip at the temperature necessary to produce decarburization, for the required length of time, the strip is trained alternately over conveyor rolls 13 in an upper series designated 13<sup>a</sup> and a lower series designated 13<sup>b</sup>.

The rolls 13 have shafts 14 extending through the side walls of the furnace and journaled in any suitable bearings carried thereby.

The shafts are driven in the known manner by any convenient mechanism.

The arrangement of the rolls in the two series as shown is such that the strip, when properly trained

thereover is caused to make a plurality of passes upwardly and downwardly throughout substantially the full height of the chamber.

The cylindrical bodies of rolls 13 may be fabricated from steel plate.

Instead of a unitary cylinder, the roll bodies may consist of a plurality of discs

spaced along the shaft.

A manifold or nozzle pipe 15 is disposed adjacent each roll 13, preferably in the V between the cylindrical roll body and the portion of the

strip 16 approaching it. The manifolds 15 are

connected by piping to any suitable source of reducing gas (not shown) and are provided with outlet ports 17 spaced therealong. The manifolds are preferably of heat-resistant alloy and are positioned so that their ports discharge jets of reducing gas onto the surface of the strip ahead of the point of contact thereof with the rolls. Any suitable means may be provided for supporting the manifolds in the proper position relative to the conveyor rolls 13, such as brackets of heat-resistant metal.

The reducing gas may be of any desired character depending on the available sources. Hydrogen is particularly effective. Carbon monoxide and methane may also be used where their carburizing property is not objectionable. Cracked ammonia gas containing about 75% hydrogen and 25% nitrogen serves very satisfactorily but the gas must have a net reducing effect since tests with neutral gas such as nitrogen do not give the desired result in preventing roll pick-up.

The reducing gas appears to exert a two-fold effect in that it tends to reduce any oxides present on the strip which are the source of roll pick-up, and also locally cools any unreduced oxides below the temperature at which they adhere to the rolls. The reducing gas should not be supplied in sufficient quantity to alter the normally slightly oxidizing character of the furnace atmosphere as a whole, which is necessary to effect the decarburization desired in the case of silicon-steel strip.

Experience indicates that the invention permits furnace rolls to operate without objectionable pick-up for periods up to one hundred times as great as those in which pick-up would otherwise occur to such an extent as to cause dimpling of the strip. The invention thus has the advantage of greatly reducing the loss of production and the expertise involved in shutting down strip-annealing furnaces for cleaning pick-up from the conveyor rolls thereof.

Although we have disclosed herein the preferred embodiment of our invention, we intend to cover as well any change or modification therein which may be made without departing from the spirit and scope of the invention.

We claim:

In a method of annealing silicon-steel strip which, at annealing temperatures, leaves accumulations of mixed oxides of iron and silicon adhering to conveyor rolls over which it travels, the steps including passing the strip through a heating zone containing a normally oxidizing atmosphere, over supporting rolls, and introducing a reducing gas directly into the V-shaped spaces between the surfaces of the rolls and the portions of the strip approaching them, at a plurality of points spaced across the width of the strip, thereby inhibiting the deposit of oxides on the rolls by the strip, and controlling the amount of reducing gas supplied so as to leave the atmosphere of said zone generally oxidizing in character.

DAVID C. BLAIR.  
HARRY F. SHANNON.

25 References Cited in the file of this patent

UNITED STATES PATENTS

| Number    | Name    | Date          |
|-----------|---------|---------------|
| 1,808,152 | Baily   | Jan. 2, 1931  |
| 1,905,809 | Cowan   | Apr. 25, 1933 |
| 2,023,285 | Otis    | Dec. 3, 1935  |
| 2,180,376 | Vaughan | Nov. 21, 1939 |
| 2,181,093 | Ness    | Nov. 21, 1939 |
| 2,232,391 | Keller  | Feb. 18, 1941 |
| 2,283,798 | Déland  | May 19, 1942  |
| 2,319,302 | Cook    | May 18, 1943  |
| 2,333,579 | Renkin  | Nov. 2, 1943  |

FOREIGN PATENTS

| 40 Number | Country       | Date          |
|-----------|---------------|---------------|
| 1,771     | Great Britain | Apr. 13, 1882 |